

July 5, 1938.

H. HIEMENZ

2,123,138

PRODUCTION OF MAGNETIZABLE MATERIALS

Filed April 2, 1936



Inventor:

Hans Hiemenz

Paul Kirkland  
Attorney

## UNITED STATES PATENT OFFICE

2,123,138

## PRODUCTION OF MAGNETIZABLE MATERIALS

Hans Hiemenz, Hanau-on-the-Main, Germany

Application April 2, 1936, Serial No. 72,364  
In Germany April 8, 1935

5 Claims. (Cl. 148—12)

This invention relates to the production of magnetizable materials containing nickel and iron which are distinguished by a constant and stable permeability, i. e. a permeability independent of the field intensity, unsensible to shocks of a direct current and amounting to as high as possible absolute values. In this direction different proposals have been made; for instance one has proposed to influence the magnetic properties by different degrees of cold-molding, for instance, cold-rolling. E. g. to obtain a high stability one has proposed to provide a double cold-molding with intermediary annealing between the cold-molding steps, relatively large reductions of the cross-section being accomplished in both cold-molding steps. It is true that a satisfactory stability of the permeability is obtained in this way, but not yet sufficiently high values of the permeability, as, for instance, required for the cores of Pupin coils which are to have as small a volume as possible, or for the continuous loading of cables. Finally for materials used in the teletransmission industry not only their qualities as to permeability are important, but on the other hand their hysteresis number, i. e. the resistance loss caused by hysteresis must be as small as possible. The hysteresis number is usually measured in ohms per henry and per ampere-winding/cm. at 800 Hertz.

A minimum value of the hysteresis number is desirable in order to reduce to a minimum the so called quality number, i. e. the quotient of the hysteresis number divided by the square root of the permeability.

According to the present invention the combination of high permeability, high constancy and stability of the permeability and small hysteresis number is obtained by dividing the cold molding into two steps in such a manner that the strip or wire is brought to 20-100 times its original length in the first operation and the product of this operation to 1.06-1.35 times its length in the second operation.

The temperature and the duration of the annealing operation between the two cold-molding steps depend upon the composition of the material used. As an approximation it may be stated that the temperatures will lie within the limits of 900 to 1200° C., the preferred temperature being 1100° C. The duration of the annealing operation preferably amounts to no more than 30 minutes and may even be less than one minute. In the most cases it is recommendable to cool down the material from the annealing temperature rapidly, for instance, by passing the strip to be heated through an annealing furnace or by quenching it in water.

By the above described treatment permeability values of from 80 to 130 are obtained, the stability and constancy of the permeability being quite satisfactory.

The double cold-molding may be combined with rolling the material down to a thickness at which the permeability in its dependency on the thickness of the strip or wire has already passed the minimum. For explanation it may be added, that when starting from a thickness of a strip or a sheet of 0.5 mm. for instance, the initial permeability decreases with decreasing thickness, passes a minimum and finally increases when the strips or sheets have become very thin, for example thinner than 0.05 or 0.03 mm.

To increase the resistance of the products, from 0.1 to 16% of suitable elements such as copper, manganese, titanium, aluminum, chromium, tungsten, molybdenum, vanadium, silicon may be added to the material to be treated.

The annexed drawing shows how the permeability  $\mu$  and the hysteresis number  $h$  depend from the extent of the second cold-molding operation in the case of an alloy of 50% iron and 50% nickel. It appears from this diagram that really on lengthening the strip or wire within the range of about 1.35 times at most the initial length extremely high values of permeability are obtained, whereas on further lengthening the values of permeability continuously decrease. The third curve finally shows the values of the quality number

$$\frac{h}{\sqrt{\mu}}$$

It appears that this value which should be as small as possible is yet satisfactory within the range indicated for the second cold-lengthening, in spite of the high values of permeability.

The course of the  $\mu$ ,  $h$  and

$$\frac{h}{\sqrt{\mu}}$$

curves in dependency on the lengthening during the second cold-molding operation varies to a certain extent with the composition of the alloys.

I claim:

1. The method of producing magnetizable materials consisting of nickel 35 to 60 parts besides iron 65 to 40 parts and having a constant and stable permeability, especially with high absolute values of the permeability, in the range of weak magnetic fields, which method consists in firstly cold-molding the magnetic material, which is, as usual in the art of cold molding, in a cast, hot-rolled or annealed condition, to about 20 to 100

5

15

20

15

25

30

35

40

45

50

55

times its initial length, then annealing the material at a temperature exceeding 900° C. and finally cold-molding the same to 1.06 to 1.35 times its length.

5      2. The method of producing magnetizable materials consisting of nickel 35 to 60 parts besides iron 65 to 40 parts and having a constant and stable permeability, especially with high absolute values of the permeability, in the range of weak 10 magnetic fields, which is, as usual in the art of cold molding, in a cast, hot-rolled or annealed condition, which method consists in firstly cold-molding the magnetic material to about 20 to 100 15 times its initial length, then annealing the material at temperatures between about 900 and 1200° C. for a period not exceeding thirty minutes, and finally cold-molding the same to 1.06 to 1.35 times its length.

20     3. The method of producing magnetizable materials consisting of nickel 35 to 60 parts besides iron 65 to 40 parts and having a constant and stable permeability, especially with high absolute values of the permeability, in the range of weak 25 magnetic fields, which method consists in firstly cold-molding the magnetic material, which is, as usual in the art of cold molding, in a cast, hot-rolled or annealed condition, to about 20 to 100 times its initial length, then annealing the material at a temperature exceeding 900° C., then rapidly 30 idly cooling down the material and finally cold-

molding the same to 1.06 to 1.35 times its length.

4. The method of producing magnetizable materials consisting of nickel 35 to 60 parts besides iron 65 to 40 parts and having a constant and stable permeability, especially with high absolute 5 values of the permeability, in the range of weak magnetic fields, which method consists in firstly cold-molding the magnetic material, which is, as usual in the art of cold molding, in a cast, hot-rolled or annealed condition, to about 20 to 100 10 times its initial length, then annealing the material for a period not exceeding one minute at a temperature exceeding 900° C., then rapidly cooling down the material and finally cold-molding the same to 1.06 to 1.35 times its length. 15

5. The method of producing magnetizable materials consisting of nickel 35 to 60 parts besides iron 65 to 40 parts and having a constant and stable permeability, especially with high absolute 20 values of the permeability, in the range of weak magnetic fields, which method consists in firstly cold-molding the magnetic material, which is, as usual in the art of cold molding, in a cast, hot-rolled or annealed condition, to about 20 to 100 25 times its initial length, then annealing the material at a temperature exceeding 900° C., then rapidly cooling down the material by passing it through an annealing furnace, and finally cold-molding the same to 1.06 to 1.35 times its length. 30

HANS HIEMENZ. 30